

## UNITED STATES PATENT OFFICE.

FREDERICK M. BECKET, OF DOUGLASTON, NEW YORK, ASSIGNOR TO ELECTRO METAL-LURGICAL COMPANY, OF NEW YORK, N. Y., A CORPORATION OF WEST VIRGINIA.

## COMPOSITION FOR TREATING METAL BATHS AND METHOD OF MAKING THE SAME.

No Drawing.

Application filed September 3, 1921. Serial No. 498,447.

This invention relates to the addition, to molten metal baths, of substances adapted to destroy or otherwise remove deleterious ingredients contained therein, or to add ingredients thereto, or otherwise to modify the properties of the molten metal and the solid metal to be produced therefrom. The invention comprises methods of adding modifying materials to metal baths, compositions to be added, and methods of preparing such compositions. The object of the invention is to improve the methods and compositions heretofore employed for the purposes to which the invention relates.

The introduction into metal baths of materials adapted to improve the quality of the metal is often attended with difficulty. Many addition agents are subject to the defect of low density. With such agents the proportion of the material actually incorporated into the bath as distinguished from being consumed by oxidation at the surface, or absorbed into the slag, is a matter of doubt, because of the tendency of the materials to float on the molten metal. I have found that lead is admirably adapted for use in conjunction with such addition agents as its high density enables it to give weight to compositions containing ingredients which are too light.

Lead also has very desirable qualities as a bonding agent for addition agents which are in comminuted form. Its softness and malleability enable it to bind such materials into coherent form, this being accomplished for example by mixing the comminuted material with lead in suitable shapes and sizes, and pressing the mixture. Briquetting is, of course, desirable, as comminuted materials tend to float because of the surface tension of the bath, and when floating and in a fine state of division, are extremely susceptible to atmospheric oxidation and other destructive influences. The bonding action of lead may also be utilized by alloying it with other addition agents, or by disseminating the latter in divided form throughout a matrix of lead or a lead alloy, as more fully described below.

Certain addition agents or scavengers, such as magnesium, are subject to the defect that their action is too energetic, so that it cannot be utilized to the best advantage. With such agents, a diluent is desirable, and

lead, being comparatively inert and assuming the liquid state at a temperature below those at which most scavengers begin to act, is well adapted to moderate the action of agents of too intense activity. Another aspect of the same effect is the protection against atmospheric oxidation at the surface of the bath which is afforded by lead. Such readily oxidizable substances as magnesium require such protection, even when they are so agglomerated and weighted that they sink into the bath in a minimum time.

The action of lead in promoting fluidity in suspended slag is especially advantageous where a scavenger is employed which, in its scavenging action, gives rise to a solid or liquid substance in the bath, which substance is incapable of combining with the bath but is adapted to unite with lead oxide to form a relatively fluid compound. Silicon may be mentioned as an example of such a scavenger. This element is frequently added to metal baths, for example as an alloy, to remove oxygen and other impurities. The oxygen compound formed therefrom combines with lead oxide to produce a fusible glass and lead is therefore a particularly valuable auxiliary agent for use in connection with silicon deoxidizers.

Lead may also be alloyed with other addition agents. A lead-magnesium alloy is an excellent form in which to add magnesium to steel or other molten metal, the lead giving the weight which the magnesium lacks, protecting the magnesium from oxidation at the surface of the bath, and diluting the magnesium so as to moderate its action on the metal. The density of the alloy can be adjusted by varying its composition, and the alloy need only be cast or cut into slugs of convenient size to prepare it for use. The alloy may have a density higher or lower than that of the metal to be treated, depending on the method of using the alloy. The following example will serve to illustrate the use of a lead-magnesium alloy:

*Example I.*—1% of an alloy containing 92% lead and 8% magnesium was added to a chrome-iron alloy, the transverse breaking test of the solidified metal showing an increase of 20% in strength over a parallel test ladle deoxidized with aluminum. The metal contained no lead and only a trace of magnesium.

In making briquets of comminuted addition agents, using lead as a binder, the latter may take the form of shot, foil, wire, chips, shavings or the like. When suitably mixed with the main addition agent or agents and subjected to pressure, a compact aggregate of regulatable density is formed, as illustrated by the following example:

*Example II.*—10 parts of magnesium shavings are mixed with 56 parts of lead shot and 34 parts of powdered manganese-silicon containing about 45% silicon and about 55% manganese, and the mixture is pressed into briquets. In this composition, both the magnesium and the lead act as binders, while the lead weights and dilutes both the other ingredients and protects them from oxidation at the surface of the bath. In accordance with the theory already set out, it is believed that the lead gives rise to substances in the bath which combine with the silica formed by the deoxidizing action of the manganese-silicon, and that the cleansing of the metal is thereby rendered more rapid and complete.

A comminuted addition agent incapable of complete alloying with lead, may be mixed with molten lead and the latter caused to solidify with unalloyed particles disseminated through it. The lead may also be replaced by a lead alloy, for example, a lead-magnesium alloy. Some care is necessary to prevent segregation of the powdered matter, but segregation may be substantially prevented by reducing the powder to proper fineness and limiting the quantity used. A very effective measure for preventing segregation when an alloy is the suspensory medium, is to adjust the density of the suspensory alloy so that it is a little less than that of the material to be disseminated through it. This can be done, in most cases, by regulating the proportion of the constituents in the alloy. The following examples are cited:

*Example III.*—Into a molten alloy containing 17 parts of magnesium and 56 parts of lead, there are stirred 27 parts of the manganese-silicon referred to in Example II, the manganese-silicon being reduced to such fineness that there is little or no segregation of the manganese-silicon on solidification.

*Example IV.*—50 parts of powdered 80% ferro-manganese are similarly mixed with a molten alloy containing 16 parts magnesium and 33 parts of lead.

From the figures given in Examples II and III, and the disclosure in my United States Patent No. 1,461,643, dated July 10, 1923, it will be apparent that in the final compositions obtained in these examples, manganese, silicon, and magnesium are present in proportions which could not be pre-

sent in a ternary alloy of these three elements. It is often desirable to add, as a single composition, the three elements referred to in amounts outside their alloying range. The compositions herein described afford a very convenient means for effecting such additions.

In the foregoing description I have referred to lead as an auxiliary agent, valuable because it enables the materials with which it is associated better to perform the functions for which they are intended. Since lead does not alloy with steel, nor with ferrous alloys in general, when such are treated with compositions containing lead no lead will remain in the bath as alloy. At the temperature of a steel bath, lead is rapidly volatilized and will therefore be boiled off or fixed in the slag. Under such conditions it will be seen that the lead does not contaminate the metal treated. I believe that the lead itself has a distinctly favorable action on the bath, as the rising lead vapors agitate the liquid metal and tend to promote the flotation of slag particles by enabling them to extricate themselves from the molten metal.

Agitation tends to liberate gases dissolved in the metal. In addition the lead vapor, upon reaching the surface of the bath and coming into contact with the air, will be oxidized; and the oxid so formed will combine with the floating slag, increasing its mobility and hence its purifying and protecting action on the bath.

While I have given what seems to me the most probable explanation of the beneficial action of the compositions described therein, this is merely by way of illustration and my invention is in no way dependent on the correctness of the explanation so given.

While the presence of lead in the composite material is preferable in many cases, it can also be omitted, especially since magnesium in the form of coarse powder or shavings is a good bonding agent for comminuted materials when the latter are mixed with the magnesium and the mixture subjected to pressure. A mixture containing magnesium, silicon and manganese, outside their allowing proportions and free from lead, is here cited as—

*Example V.*—20 parts of magnesium, as coarse powder or shavings, are mixed with 80 parts manganese-silicon of the composition given under Example II and the mixture pressed into briquets of convenient size. The magnesium is a sufficient binder, especially when used as shavings, and the manganese-silicon serves to weight, protect and dilute the magnesium.

As disclosed in Patent 1,322,158 granted to me Nov. 18, 1919, it is advantageous when magnesium is used as a cleansing agent for

metal baths to use silicon in conjunction therewith, in order that a fusible product may be formed by the action of the composition on the metal to which it is added. 5 The addition of manganese to the magnesium and silicon is also disclosed, the three elements being formed into an alloy. Other alloys containing these three elements are disclosed in my United States Patent No. 10 1,461,643 referred to above. In the use of all these compositions, the acidic oxides formed from the silicon combines with the basic oxides formed from the magnesium and the manganese, giving fusible slags. Silicon 15 has a similar fluxing action when used in conjunction with other metals forming basic oxides, such metals being in general the chemical elements which are more electro-positive than silicon. 20 When it is desired to use silicon with metallic addition agents for its fluxing action, it is often found that the proportions which appear most desirable are outside the alloying limits. In such cases, unalloyed or 25 incompletely alloyed compositions may be prepared in accordance with the present disclosure.

I am aware that various known addition agents for steel baths, for example commercial ferro-manganese, are not strictly homogeneous in their microstructure, containing 30 undissolved microscopic particles of carbids and the like. Such compositions falling within my invention as are incompletely alloyed, are distinguished from these materials in that such incompletely alloyed compositions as are herein claimed contain 35 considerable quantities of macroscopic particles, suspended in a matrix of solidified metal, or 40 bonded with a compacted metallic binder.

While I have described my invention in connection with certain specific materials and methods, these are cited merely for illustration, and the scope of my invention is 45 defined only by the appended claims.

I claim:

1. A composition for treating metal baths, comprising in coherent form a main addition agent existing in macroscopic particles 50 and a soft, relatively heavy, low-melting and relatively inert metallic binder.
2. A composition for treating metal baths, comprising in coherent form a main addition agent existing in macroscopic particles 55 and a metallic binder comprising lead.
3. A composition for treating metal baths, comprising in coherent form a main addition agent and a metallic binder comprising magnesium and lead. 60
4. A composition for treating metal baths, comprising in coherent form a main addition agent and a metallic binder comprising an alloy of magnesium and lead. 65
5. A composition for treating metal baths, comprising in coherent form a silicon alloy

existing in macroscopic particles and a metallic binder comprising lead.

6. A composition for treating metal baths, comprising in coherent form a silicon alloy 70 existing in macroscopic particles and a metallic binder comprising magnesium and lead.

7. A composition for treating metal baths, comprising in coherent form a silicon alloy 75 existing in macroscopic particles and a metallic binder comprising an alloy of magnesium and lead.

8. Method of forming a scavenging composition for metal baths, which comprises adding to molten metals, particles of an addition agent incapable of completely dissolving in said molten metal, and then cooling the metal to solidification. 80

9. Method of forming a scavenging composition for metal baths, which comprises 85 adding to molten metal containing lead, particles of an addition agent incapable of completely dissolving in said molten metal, and then cooling the metal to solidification.

10. Method of forming a scavenging composition for metal baths, which comprises adding to a molten lead-magnesium alloy, 90 particles of a silicon alloy incapable of completely dissolving in said molten alloy, and then cooling the molten alloy to solidification. 95

11. Method of forming a scavenging composition for metal baths, which comprises adding to a molten alloy containing a light metal, particles of an addition agent incapable of completely dissolving in said 100 molten alloy, said addition agent having a higher density than said light metal, and the content of said light metal in said molten alloy being so adjusted that the molten alloy 105 has a lower density than said addition agent.

12. Method of scavenging metal baths, which comprises adding thereto magnesium alloyed with a metal adapted to volatilize in the bath. 110

13. Method of scavenging metal baths, which comprises adding thereto magnesium alloyed with a metal adapted to volatilize in the bath and to increase the fluidity of the slag. 115

14. Method of scavenging metal baths, which comprises adding thereto a composition comprising an alloy containing magnesium and a metal of a materially higher density than the metal of the bath, and adjusting the proportions of the constituents of the composition so that the composition will have a density higher than that of the bath. 120

15. Method of scavenging steel baths, which comprises adding thereto an alloy containing lead and a more active deoxidizer. 125

16. Method of scavenging steel baths, which comprises adding thereto a magne- 130

sium alloy having a higher density than that of the bath, said alloy containing a volatile metal.

17. Method of scavenging steel baths, which comprises adding an alloy of lead and magnesium thereto.

18. Method of treating molten metal, which comprises adding thereto lead and an addition agent capable of forming an oxidation product which combines with the oxid of lead to form a fusible slag.

19. Method of treating molten steel, which comprises adding thereto lead and an addition agent capable of forming an oxidation product which combines with the oxid of lead to form a fusible slag.

20. The method of treating molten iron or steel comprising incorporating therewith a

material containing magnesium and having a specific gravity higher than the molten iron or steel.

21. The method of treating molten iron or steel comprising incorporating therewith a material containing magnesium and lead.

22. The method of treating molten iron or steel comprising incorporating therewith a material containing magnesium and lead and having a specific gravity higher than the molten iron or steel.

23. The method of treating molten iron or steel comprising incorporating therewith an alloy containing magnesium and lead and having a specific gravity higher than the molten iron or steel.

In testimony whereof, I affix my signature.  
FREDERICK M. BECKET.